

June 8, 1926.

1,587,944

H. W. FLETCHER  
LUBRICANT COMPOSITION FOR THE BEARINGS OF THE CUTTERS ON A ROLLER  
EARTH BORING DRILL  
Filed Jan. 25, 1921



Fig. 1.



Fig. 2.

H. W. FLETCHER, INVENTOR.

BY *Jesse R. Stone*

ATTORNEYS.

Patented June 8, 1926.

1,587,944

# UNITED STATES PATENT OFFICE.

HAROLD W. FLETCHER, OF HOUSTON, TEXAS, ASSIGNOR TO HUGHES TOOL COMPANY,  
OF HOUSTON, TEXAS, A CORPORATION OF TEXAS.

## LUBRICANT COMPOSITION FOR THE BEARINGS OF THE CUTTERS ON A ROLLER EARTH-BORING DRILL.

Application filed January 25, 1921. Serial No. 439,738.

My invention relates to a lubricating composition for especial application to rotary earth boring drills of the roller type. In such devices the drill bits used have cutting 5 rollers on the forward end thereof that are adapted to roll on the bottom of the hole and act to disintegrate the material. Streams of flushing fluid are pumped down from the surface through the hollow drill 10 stem to which the bit is attached. This fluid is discharged through channels in the head of the bit upon the cutters and serves to wash away the disintegrated matter and carry it in suspension up outside the drill 15 stem to the surface where it is discharged.

The rolling cutters which act to drill the hole are under heavy strain and also operate under the pressure of a head of mud in the hole. The type of lubricator best adapted 20 to work under these conditions is disclosed in Hughes Patent No. 930,759 issued August 10, 1909. The head of water in the drill stem is slightly in excess of the head of water outside of the drill stem due to the 25 pressure of the pumps and to the damming up of the water in the drill stem by the relatively small passages in the head of the bit through which the flushing fluid is discharged. This excess pressure is exerted 30 upon the lubricant in its container and serves to force it to the bearings against the slightly smaller head of fluid pressure outside the drill stem.

The difficulty with this method of lubrication is that it is rather difficult to fit a plunger over the lubricant in its container which will move freely and still be tight enough to prevent the muddy flushing fluid, which drives the lubricant, from leaking 35 past the plunger to mix with the lubricant in the container. It is found that the mud after thus finding entrance to the lubricant will, because of its greater specific gravity, sink to the bottom of the lubricator and thus 40 pass directly to the bearings of the cutting rollers and destroy the lubrication.

An object of my invention is to provide 45 a method of treating the lubricant for use in roller earth boring drills so that the mud will not mix with the lubricant and pass therethrough to the bearings.

Another object is to prevent the mixture 50 of the flushing fluid, used with earth boring drills, with the lubricant by making the

lubricant of heavier specific gravity than is 55 the flushing fluid.

Referring to the drawings, I have illustrated in Fig. 1 a view, partly in central longitudinal section, showing a roller drill in which ordinary lubricant is used. Fig. 60 2 is a similar view in which the effect of my improved method of lubrication is shown. Like numerals of reference apply to like parts in both the views.

The drill 1 is shown in the drawing as 65 having roller cutters 2 on the forward end thereof. The drill is attached by means of a drill collar 3 to a drill stem 4 by means of which it is rotated by mechanism at the surface of the ground.

A lubricator, consisting of a barrel 5 of 70 relatively small diameter, is secured to a nipple 6 on the upper shank of the bit. Passages or oil ducts, not shown, lead from the lubricator through the head to the bearings of the drill as shown in the Hughes 75 patent previously referred to. The upper end of the lubricator is closed by a plug 7 screwed internally within the barrel. Below the plug, openings 8 allow entrance of 80 flushing fluid to the interior of the lubricator barrel.

Within the lubricator a plunger 9 rests 85 upon the upper surface of the lubricant 10 and serves to transmit the pressure of the 85 flushing fluid to the lubricant to force said lubricant to the bearings of the cutters.

In the operation of the device as shown in 90 Fig. 1 the lubricant is a heavy grade of lubricating oil. No specific grade of lubricant is required, but I have used an oil having a specific gravity of about 0.9, a flash point of approximately 400° Fahrenheit, and a viscosity of around 500 Saybolt, or 95 over. The spots 11 indicate small masses of the flushing fluid which have been forced past the plunger and the masses are slowly sinking to the lower end of the lubricator end to the bearings of the cutters.

To avoid this mixing of the mud with the 100 oil, I contemplate compounding with the lubricant a pulverized heavy mineral substance such as lead oxide or barium sulfate, which will stay in suspension in the lubricant and will not affect the lubricating 105 qualities of the oil. This mixture of lubricant and heavy mineral will have a greater specific gravity than the flushing fluid. For

this reason, if the flushing fluid works past the plunger, it will still stay on top of the lubricant as indicated in Fig. 2 and will not affect the lubrication of the cutter bearings 5 until the lubricant itself has been entirely exhausted. As it is possible to regulate the size of the lubricator and the quantity of lubricant therein to provide an amount sufficient to run for the desired length of time, 10 no trouble with muddy lubricant will be experienced. Barium sulfate is especially adapted for mixing with the lubricant. It remains readily in suspension and is of high molecular weight. Furthermore it does not 15 affect the lubricating qualities of the oil detrimentally. With the use of this method no plunger need be employed at all unless so desired, the result being the same.

The value of my method of lubrication 20 under the conditions in which earth boring drills operate, lies largely in its simplicity. Lack of skill on the part of the driller in fitting the plunger or in screwing the cap on the lubricator or otherwise will not re-

sult disastrously. It is only necessary to 25 mix with the lubricant a suitable proportion of the heavy mineral in the manner described and the greater specific gravity of the lubricant will prevent the mixture therewith of the flushing mud and thus prevent 30 wear on the bearings.

Having thus described my invention, the advantages of which will be apparent to one skilled in the art, what I claim as new and desire to protect by Letters Patent is: 35

A lubricant for the bearings of the cutters on a roller earth-boring drill in which a muddy fluid is used in forcing the same to the bearings, consisting of a mixture of heavy grade lubricant with a heavy pulverized mineral substance in quantities sufficient to raise the specific gravity above that of said muddy fluid. 40

In testimony whereof, I hereunto affix my signature, this the 15th day of January, A. 45 D., 1921.

HAROLD W. FLETCHER.